

P. A. E. ARMSTRONG.

PROCESS OF PREVENTING CORES FOR TUBULAR BODIES FROM WELDING.

APPLICATION FILED JAN. 17, 1919.

1,341,204.

Patented May 25, 1920.



FIG. 3



INVENTOR  
P.A.E. Armstrong  
BY  
H.H. Dyke  
ATTORNEY

# UNITED STATES PATENT OFFICE.

PERCY A. E. ARMSTRONG, OF LOUDONVILLE, NEW YORK.

## PROCESS OF PREVENTING CORES FOR TUBULAR BODIES FROM WELDING.

1,341,204.

Specification of Letters Patent. Patented May 25, 1920.

Application filed January 17, 1919. Serial No. 271,611.

*To all whom it may concern:*

Be it known that I, PERCY A. E. ARMSTRONG, a subject of the King of Great Britain, and a resident of Loudonville, county of Albany, and State of New York, have invented certain new and useful Improvements in Processes of Preventing Cores for Tubular Bodies from Welding, of which the following is a specification.

10 The present invention relates to the making of tubular bodies, such as steel drill rod and the like, in which a metallic core is inserted in the bore of a longitudinally bored billet and the billet and core are worked for 15 elongation and reduction of cross section, as by rolling after which the core is withdrawn.

According to the present invention the core, which, in the case of making steel drill rod, may also be of steel preferably some- 20 what milder and more ductile than the drill rod steel, is coated with a layer of metal which will not melt at the temperatures used and will prevent welding taking place between the billet and core.

25 One metal well adapted for the purpose is nickel. The non-welding metallic layer may be applied in any desired way, as, for example, by plating it on the outer surface of the core or upon the walls of the billet bore, or both.

When nickel is electro-plated on steel, for example, a continuous coating may be readily obtained, but the bond between the steel and the nickel plate is not so strong as if 35 the steel is first plated with copper, for example, and the nickel plated upon the copper surface so obtained. Direct plating upon the steel is preferable for the present invention, since, so long as a continuous 40 layer of non-welding metal, such as nickel, is present between the core and the wall of the billet bore, welding will be prevented from taking place therebetween, and when it comes to withdrawing the core, such operation may be facilitated by the relative 45 weakness of the bond between the steel and the nickel layer.

In the accompanying drawing Figure 1 is a longitudinal sectional view of a longitudinally bored billet having a two-piece core therein, the core ends being shown as projecting beyond the ends of the billet. Fig. 2 is a similar view, on an enlarged scale, of the billet and core of Fig. 1 after

rolling and before withdrawal of the core, 55 and Fig. 3 is a view similar to Fig. 1, but with a one-piece core, and in this view the core ends are shown flush with the ends of the billet.

The billet 10 has a bore 11. The core 60 portions 12 and 13 of Figs. 1 and 2, and the one-piece core 14 of Fig. 3, are shown provided with a coating 15 of metal which will not melt at the temperatures used, as, for example, nickel preferably plated direct 65 upon the core, though it may be applied to the bore walls or to both core and to the bore walls. To put the core in the billet the latter is preferably heated, though this is not essential. When heating is resorted 70 to it serves to shrink the billet on the core, and further, the film of oxid formed on the bore walls serves to prevent any tendency toward union between the nickel and the iron during the rolling or other working 75 operation. The core may be fastened in place by welding it to the billet at the end or ends, if desired. Welding at one end is indicated at 16, Fig. 3.

After the billet and core have been worked 80 for elongation and reduction of cross section, as by rolling, the core is pulled out, the core of Fig. 2, parted between its ends, being pulled out from the opposite ends in two parts, and the core of Fig. 3 being pulled 85 out from one end. When the core ends project beyond the billet ends they may be seized for pulling out. If the core ends do not project beyond the billet ends the tubular body produced may be broken or cut off, 90 leaving the core end projecting for pulling out, or in case it is a core end to be pulled through the bore of the tubular body, the cut or break may extend entirely across the end, thereby removing any relatively enlarged 95 or deformed end portion of the core, which would interfere with pulling out.

It will be apparent that the invention as described is of great simplicity and that all the parts and materials involved are of 100 metallic character and readily worked in a steel mill, for example. The presence of foreign materials, such as sand, is dispensed with, and the drill rod or other tubular body produced has a smooth bore and is immediately ready for use upon withdrawal of the core and without any necessity for removal of foreign material, such as sand

and the like, and strong tubular bodies such as drill rod and the like may be produced having good bores of small diameter.

While the invention has been described with particular reference to the manufacture of steel drill rod, it is to be understood that the same may be made use of in connection with the manufacture of tubular bodies of other kinds and made from a variety of materials.

I claim:

1. The process of making tubular bodies such as hollow drill rod and the like which comprises introducing a metallic core into a bored billet with a layer of non-welding metallic material interposed therebetween, elongating and reducing the cross section of billet and core as by rolling, and withdrawing the elongated core from the tubular article produced.
2. The process of making tubular bodies such as hollow steel drill rod and the like which comprises applying a coating of non-welding metallic material to a metal core, introducing same into a bored billet, elongating and reducing the cross section of billet and core as by rolling, and withdrawing the core from the tubular body produced.
3. The process of making tubular bodies

which comprises coating a steel core with 30 nickel, introducing same in a longitudinally bored steel billet, elongating and reducing the cross section of billet and core as by rolling, and withdrawing the core from the tubular body produced.

4. The process of making tubular bodies which comprises providing a bored billet and a core body of metallic material adapted to weld together, applying to the core body a coating of non-welding metallic material, introducing the core so formed into a bored billet, elongating and reducing the cross section of billet and core as by rolling, and withdrawing the core from the tubular body produced.

5. The process of making tubular bodies which comprises coating a core body with non-welding metallic material, introducing same into a bored billet of material similar to the core body, elongating and reducing the cross section of billet and core as by rolling, and withdrawing the core from the tubular body produced.

In testimony that I claim the foregoing I have hereto set my hand, this 14th day of January, 1919.

PERCY A. E. ARMSTRONG.